

(No Model.)

C. W. HUBBARD.  
MANUFACTURE OF AXES.

No. 444,836.

Patented Jan. 20, 1891.



Fig. 1



Fig. 2.



Fig. 3.

WITNESSES.

*W. M. Clark*  
*A. G. M. Conner*

INVENTOR.

*Charles W. Hubbard*  
*by W. D. Russell & Son*  
*his Attorneys.*

# UNITED STATES PATENT OFFICE.

CHARLES W. HUBBARD, OF PITTSBURG, PENNSYLVANIA.

## MANUFACTURE OF AXES.

SPECIFICATION forming part of Letters Patent No. 444,836, dated January 20, 1891.

Application filed October 11, 1890. Serial No. 367,798. (No model.)

*To all whom it may concern:*

Be it known that I, CHARLES W. HUBBARD, of Pittsburgh, in the county of Allegheny and State of Pennsylvania, have invented a new and useful Improvement in the Manufacture of Axes, of which the following is a full, clear, and exact description, reference being had to the accompanying drawings, forming part of this specification, in which—

10 Figure 1 is a plan view of a bar of steel rolled into proper form for the manufacture of my improved poll-blank. Fig. 2 is a vertical cross-section of the bar shown in Fig. 1. Fig. 3 shows the manner in which the severed blank is bent 15 to form the ax-poll.

My invention consists in a bar of steel rolled into a certain shape in cross-section, herein-after described, and adapted when divided transversely to form blanks each of which 20 when bent together and welded constitutes an ax-poll having a finished eye or hole for the reception of the helve.

Heretofore attempts have been made to make ax-polls in this manner; but the sections 25 of the bars have been such that they have been difficult, if not impossible, of rolling and when rolled were not adapted to be shaped into a useful ax-poll.

The object of my invention is to overcome 30 the defects of such prior expedients and to provide means by which ax-poll blanks can be made by rolling in a cheap and efficient manner.

I first roll a bar of steel of the shape in cross- 35 section shown in Fig. 2, having a thick middle portion 2 and side portions 3, which extend from the middle portion in opposite di-

rections in substantially the same plane, one side of the bar being formed with plain or flat portions 4 along the margin and with a curved 40 surface between these flat portions and a concavity 5 on the inner side of the middle portion 2. Such bar of steel is easily rolled without extra labor or cost. When it is so rolled, I cut it transversely into blanks, as indicated 45 by dotted lines in Fig. 1. I then take a blank formed in this way and bend up its arms 3 toward each other, and when the flat portions 4 are brought in contact, as shown in Fig. 3, and welded, the ax-poll is completed. The 50 section of the blank is such that the ax-poll is completely shaped by bending up the sides of the blank. To this end the concavity 5 is of material importance, because if it were not present the eye of the ax would be misshapen 55 and would require special treatment to reduce it to proper form.

By modification of the shape of the head 2 the bar may be adapted to produce blanks for double-bitted axes or axes with heads of special 60 shapes.

The advantages of my invention will be appreciated by those skilled in the art.

I claim—

A rolled bar substantially of the shape in 65 cross-section shown in Fig. 2 and adapted to be divided into ax-poll blanks, substantially as and for the purposes described.

In testimony whereof I have hereunto set my hand this 9th day of October, A. D. 1890. 70

CHARLES W. HUBBARD.

Witnesses:

W. B. CORWIN,  
H. M. CORWIN.